

## 1

3,441,577

## PROCESS FOR THE CO-OLIGOMERIZATION OF CONJUGATED UNSATURATED FATTY ACIDS OR THEIR ESTERS WITH INDENE AND/OR COUMARONE

Josef Baltes, Hamburg, Friedrich Weghorst, Hamburg-Harburg, and Otto Wechmann, Westerhof, Germany, assignors to Harburger Fettschemie Brinckman & Mergell G.m.b.H., Hamburg-Harburg, Germany, a corporation of Germany  
No Drawing. Filed Mar. 22, 1965, Ser. No. 441,874  
Claims priority, application Germany, Aug. 22, 1964,  
H 53,613  
Int. Cl. C09f 7/06

U.S. CL. 260—407

9 Claims

## ABSTRACT OF THE DISCLOSURE

Conjugated unsaturated fatty acids and their esters are co-oligomerized with indene and/or coumarone at a temperature of 40 to 180° C. in the presence of an acid or Friedel-Crafts catalysts.

The present invention relates to a process for cationic co-oligomerization of conjugated-unsaturated fatty acids or their esters with indene and/or coumarone.

The conversion to coumarone resins of the light oil fractions from coal tar which are commonly designated as "Losungsbenzol II" or solvent naphthas having boiling ranges of from 150 to 200° C., and which contain considerable quantities of indene and somewhat lower amounts of coumarone with acid or Friedel-Crafts catalysts is known. It is also known to boil the coumarone resin with drying oils such as linseed and to use the boiled product as a raw material for lacquers. Furthermore, it has been proposed to react unsaturated fatty acids and drying or half-drying oils with indene by heating. The mechanism of this reaction and the chemical structure of the products obtained have been enlightened by H. P. Kaufman and H. Bruning and described in "Fette, Seifen, Anstrichmittel," 62 (1960), page 1146. According to these authors, the reaction is a diene synthesis in the sense of Diels-Alder wherein from one molecule each of indene and conjugated-unsaturated fatty acid a monocarboxylic acid derivative of tetrahydrofluorene is formed. Thus beta-eleostearic acid yields 1-(n-hexen-1'-yl)-4-(carbmetoxy-n-heptyl)-1,4,10,11-tetrahydrofluorene, and 9,12-linolic acid yields 1-n-hexyl-4-(carbmetoxy-n-heptyl)-1,4,10,11-tetrahydrofluorene. In these reactions, indene functions as a dienophilic reactant. In the case of 9,12-linolic acid, the acid is converted first to the corresponding conjugated fatty acid, which is then subjected to the diene synthesis with indene. Accordingly, it is also possible to react drying and half-drying oils containing isolated-unsaturated fatty acids in a triglyceride bond such as linseed oil, soya oil, sunflower oil and the like in the sense of this reaction mechanism by heating them with indene to elevated temperatures, whereby useful raw materials for lacquers are obtained.

N. C. Deno has proposed in "Journ. Amer. Chem. Soc." 72 (1950), page 4057, to react lower molecular unsaturated acids and their derivatives, e.g., sorbic acid and muconic acid, with indene and coumarone yielding also Diels-Alder products. Finally, it is known from German Patent 1,110,865, German application DAS 1,161,026,

## 2

and the publication by A. Henglein and H. G. Stolzenbach in "Makromolekulare Chemie," 44-46 (1961), page 138, to add acrylic acid or lower molecular dicarboxylic acid anhydrides such as maleic acid anhydride, itaconic acid anhydride and citraconic acid anhydride to indene or coumarone.

It has now been found that conjugated-unsaturated fatty acids or their esters or fatty acids or ester mixtures containing conjugated-unsaturated fatty acids can be co-oligomerized with indene and/or coumarone by cationic reaction. The process of the invention comprises reacting in the presence of an acid catalyst or catalysts of the Friedel-Crafts type one mol of the conjugated, unsaturated fatty acids or esters of the acids with from 0.5 to 20 mols of indene and/or coumarone. To prevent the formation of any free radicals which otherwise might affect the result, the reaction is conducted in the presence of a phenolic inhibitor.

According to a preferred embodiment of the process of the invention, isomerized monoesters of half-drying oils such as isomerized soya oil fatty acid methyl ester, isomerized safflower oil fatty acid methyl ester and the like containing 40 to 75% of conjugated-unsaturated fatty acid in ester bond and indene- and/or coumarone-containing hydrocarbon mixtures such as the coal tar oil fractions designated as "Losungsbenzol II" or solvent naphtha are used.

The isomerized fatty acid monoesters used as starting material are obtained from isolated-unsaturated fatty acid monoesters according to our United States Patent No. 3,162,658, Dec. 22, 1964, to which reference is made. As stated in said patent, the fatty acid ester is an ester of a hydrocarbyl alcohol having 1 to 18 carbon atoms. The fatty acid monoesters are mixed with indene and/or coumarone or the corresponding amounts of "Losungsbenzol II" in a ratio of 0.5 to 20 mols of indene and/or coumarone per mol of conjugated-unsaturated fatty acid or its monoester and heated in the presence of acid catalysts, e.g., acid activated bleaching earth, with stirring and gradual temperature increase until in the temperature range between 40° and 120° C. the co-oligomerization commences. This stage is indicated by the spontaneous temperature increase of the reaction mixture. For completion of the reaction, the mixture is heated—if necessary with a temperature increase up to a maximum of 180° C. When using "Losungsbenzol II," however, the temperature limit is its boiling point. Heating is continued under reflux until there is no change in the viscosity of the reaction mixture.

In order to eliminate the catalytic influence of peroxides and therewith a possible undesirable radical reaction, the conversion is carried out in the presence of small amounts of phenolic inhibitors such as hydroquinone, butyl catechol and the like. In general, the reaction requires 1 to 4 hours.

After the catalyst has been removed by filtration or by washing, the fatty acids which do not participate in the reaction, namely saturated and monounsaturated fatty acids, are removed by distillation under reduced pressure. When using "Losungsbenzol II" the reacted hydrocarbons derived from "Losungsbenzol II," mainly higher benzene homologues, are removed in the same manner. Depending upon the proportions of the original components, the residues are liquid to highly viscous to solid resinous homogeneous masses, which comprise in large part polybasic carboxylic acids together with monocarboxylic acids

and are characterized by their acid number or saponification number. The products obtained with a low molar ratio of the reaction components can be distilled without decomposition under high vacuum.

The process of the invention is applicable only to conjugated-unsaturated fatty acids and their esters: not to isolated-unsaturated fatty acids and their esters. Under the conditions of the process, a homo-oligomerization of the single reactants is practically excluded. This is shown by the very small amounts of unsaponifiable components present in the products obtained by the process of the invention. This, and the acid catalysts or Friedel-Crafts catalysts which are used as well as the necessity to exclude peroxides which could act as catalysts in the sense of a free-radical reaction characterize the process as a cationic co-oligomerization. Accordingly, the products obtained by the process of the invention are mixtures of isomeric mono- and polycarboxylic acids or their esters. Typical examples of such acids, starting, e.g., from 9,11-linolic acid, have the following structural formula:

I.  $\text{CH}_3-(\text{CH}_2)_6-\text{CH}-\text{CH}=\text{CH}-(\text{CH}_2)_7-\text{COOH}$



$n=0$  or integer.



$n=0$  or integer.

$\text{CH}_3-(\text{CH}_2)_6-\text{CH}-\text{CH}=\text{CH}-(\text{CH}_2)_7-\text{COOII}$



$\text{CH}_3-(\text{CH}_2)_6-\text{CH}=\text{C}-\text{CH}=\text{CH}-(\text{CH}_2)_7-\text{COOII}$

$n=$ integer.

Thus the new products obtained by the process of the invention differ substantially from the known diene products as well as from the addition products formed by radicalic reactions, which are all monocarboxylic acids.

The main advantage of the present invention is that it permits the addition of about 15 to 700 parts by weight of indene and/or coumarone to 100 parts by weight of conjugated-unsaturated fatty acids or their esters to form chemically defined mono- and polycarboxylic acids or their esters which due to their favorable properties are useful for a great variety of applications.

In contrast to coumarone resins and their hitherto known combination products with unsaturated fatty acids and drying or half-drying oils, the products obtained by the process of the invention, surprisingly, exhibit an outstanding light stability. Therefore, they are especially suitable for the manufacture of nonyellowing lacquers and coatings, the chemical and mechanical properties of which can be widely varied and adapted to the desired properties

by selection of the molar ratio of indene/conjugated-unsaturated fatty acids. A further advantage of the invention is that a ratio of 0.5 to about 2 mols indene and/or coumarone per mol conjugated-unsaturated fatty acid, oligomeric dicarboxylic acids are obtained as a main product which due to their bifunctional character are accessible to polyaddition or polycondensation and can be used therefore for the manufacture of plastics, e.g., polyamides. In the form of their hydroxy group-containing polyesters, they are especially suitable for the polyaddition with polyisocyanates, whereby rubber-like masses or foams are obtained.

#### EXAMPLE 1

600 g. of isomerized sunflower oil fatty acid methyl ester containing 65% conjugated-unsaturated fatty acid methyl ester (about 1.3 mols), 116 g. of indene (1 mol), 6 g. of acid activated bleaching earth and 0.5 g. of hydroquinone were heated with stirring in an atmosphere of nitrogen; the indene was dissolved within a short time. After the mixture had reached a temperature of about 90° C., a brownish discoloration of the catalyst was observed. At the same time, the temperature spontaneously increased to 140° C. within a few minutes. The reaction mixture was maintained at 140° C. for several hours; during this time samples for viscosity measurements were taken at half hour intervals (Höppler viscosimeter, 50° C.). In the course of one hour, the viscosity of the mixture increased continuously, whereas in the following 3 hours practically no further increase of viscosity was observed. After cooling to about 80° C. and following the removal of the catalyst by filtration, the mixture was subjected to fractional distillation to separate the fatty acid methyl esters which had not participated in the reaction. These proved to be mainly oleic acid and palmitic acid methyl esters, and possibly some unreacted indene. In a boiling range of 180° to 190° C. at an initial pressure of 5 torrs and a final pressure of 1 torr a total of 245 g. distillate corresponding to 34.2% was obtained showing a saponification number of 185 and containing 1.2% of unsaponifiable matter. The distillation residue weighing 470 g. corresponding to 65.8% had a saponification number of 146 and contained 2.2% of unsaponifiable. The free total fatty acids recovered from a part of this residue had a saponification number of 156. 100 g. of the distillation residue were subjected to fractional distillation at 0.1 torr. The boiling ranges and characteristics of the single fractions are shown in the following table:

|                   | Boiling Range<br>°C. | Quantity,<br>grams | Saponification<br>Number | $H_{D45}^{\circ} \text{C}$ |
|-------------------|----------------------|--------------------|--------------------------|----------------------------|
| Fraction I.....   | 204-257              | 18.8               | 143.5                    | 1.4938                     |
| Fraction II.....  | 257-287              | 19.1               | 153                      | 1.4959                     |
| Fraction III..... | 287-310              | 20                 | 153                      | 1.4969                     |
| Fraction IV.....  | 310-325              | 19.1               | 145.8                    | 1.5022                     |
| Fraction V.....   | 325-345              | 9.1                | 144                      | 1.5058                     |
| Residue.....      |                      | 13.9               | 131                      | -----                      |

#### EXAMPLE 2

In this example, "Losungsbenzol II" having a boiling range of 175° to 201° C. and containing 63.3% polymerizable matter comprising a major portion of indene and a minor portion of coumarone was used together with isomerized safflower oil methyl ester containing 66% of conjugated-unsaturated fatty acid methyl ester. The catalyst used was acid activated bleaching earth in an amount of 2%, based on the total batch, and the inhibitor used was di-tert.-butyl-p-cresol (0.05%). The reaction time amounted to 4 hours and the reaction temperature was held to 180° C. max. All other working conditions were the same as used in Example 1 with the exception that, when distilling the co-oligomerisate, the hydrocarbons and fatty acid methyl esters were recovered in separate fractions. The following table shows typical batches

with varied molar ratios of the reactants, the yields obtained and the characteristics of the products:

| Batch<br>(a) g. of ester<br>(b) g. of "Losungs-<br>benzol II" | Molar Ratio<br>of indene/<br>conjugated-<br>unsaturated-<br>fatty acid | abt. 1:2   | Percent Yield                    |                                            |                      | Saponi-<br>fication<br>Number |
|---------------------------------------------------------------|------------------------------------------------------------------------|------------|----------------------------------|--------------------------------------------|----------------------|-------------------------------|
|                                                               |                                                                        |            | (a) hydrocarbon                  | (b) monomeric                              | F.A. esters          |                               |
|                                                               |                                                                        |            | (c) co-oligomeric<br>F.A. esters | Consistency<br>(softening<br>point in °C.) |                      |                               |
| (a)                                                           | 600                                                                    |            |                                  | 6                                          | Liquid-----          |                               |
| (b)                                                           | 117                                                                    |            | (b)                              | 25                                         | -----do-----         | 175.5                         |
|                                                               |                                                                        |            | (c)                              | 65                                         | -----do-----         | 165                           |
| (a)                                                           | 600                                                                    | abt. 1:1.4 | (a)                              | 9                                          | Liquid-----          |                               |
| (b)                                                           | 185                                                                    |            | (b)                              | 29                                         | -----do-----         | 168                           |
|                                                               |                                                                        |            | (c)                              | 63                                         | -----do-----         | 152.3                         |
| (a)                                                           | 600                                                                    | abt. 1.5:1 | (a)                              | 14                                         | Liquid-----          |                               |
| (b)                                                           | 390                                                                    |            | (b)                              | 22                                         | -----do-----         | 160                           |
|                                                               |                                                                        |            | (c)                              | 64                                         | Viscous-----         | 92                            |
| (a)                                                           | 300                                                                    | abt. 7:1   | (a)                              | 31                                         | Liquid-----          |                               |
| (b)                                                           | 910                                                                    |            | (b)                              | 7                                          | -----do-----         | 111.5                         |
|                                                               |                                                                        |            | (c)                              | 62                                         | Semi-solid (20)----- | 63.9                          |
| (a)                                                           | 154                                                                    | abt. 13:1  | (a)                              | 32                                         | Liquid-----          |                               |
| (b)                                                           | 800                                                                    |            | (b)                              | 6                                          | -----do-----         | 98.5                          |
|                                                               |                                                                        |            | (c)                              | 62                                         | Solid (60)-----      | 44.4                          |
| (a)                                                           | 77                                                                     | abt. 20:1  | (a)                              | 33                                         | Liquid-----          |                               |
| (b)                                                           | 900                                                                    |            | (b)                              | 3                                          | Viscous-----         | 55.7                          |
|                                                               |                                                                        |            | (c)                              | 64                                         | Solid (87)-----      | 25                            |

We claim:

1. Process for the cationic co-oligomerization of conjugated, unsaturated fatty acids with a compound selected from the class consisting of indene, coumarone, and mixtures thereof, which comprises reacting a substance selected from the class consisting of conjugated, unsaturated fatty acids and esters of such acids with hydrocarbyl alcohols having 1 to 18 carbon atoms in the proportions of 1 mol of said acid substance to from 0.5 to 20 mols of the said indene and/or coumarone compound, conducting the reaction at temperatures from 40 to 180° C. in the presence of a catalyst selected from the group consisting of acid and Friedel-Crafts catalysts, and a phenolic inhibitor of free-radical reaction, for a time sufficient to bring about a stable, increased viscosity in the reaction mass.

2. Process according to claim 1 wherein the reaction is caused to take place under an inert atmosphere.

3. Process according to claim 1 wherein, following the reaction, the catalyst is separated from the reaction mass and thereafter, the catalyst-free mass is subjected to distillation under reduced pressure to remove non-reacted components.

4. Process according to claim 1 wherein the conditions establishing cationic co-oligomerization are secured by conducting the reaction in the presence of a catalytic amount of an acid-treated bleaching earth catalyst, and free-radical type reaction is inhibited by the presence of an effective fractional percent of a phenolic inhibitor se-

lected from the class consisting of hydroquinone, butyl catechol, and di-tertiary-butyl-para-cresol.

25 5. A process according to claim 1 wherein said substance is a methyl ester.

6. A process according to claim 5 wherein said substance is a member of the group consisting of the methyl ester of isomerized soya oil fatty acids, isomerized safflower oil fatty acids and isomerized sunflower oil fatty acids.

30 7. A process according to claim 1 wherein said compound is indene.

8. A process according to claim 1 wherein said compound is coumarone.

35 9. A process according to claim 1 wherein said compound is a mixture of indene and/or coumarone.

#### References Cited

##### UNITED STATES PATENTS

40 3,271,432 9/1966 Baltes et al. ----- 260—407

##### FOREIGN PATENTS

950,602 2/1964 Great Britain.

1,007,914 10/1957 Germany.

##### 45 OTHER REFERENCES

Kaufman et al.: Fette. Seifen. Anstrichmittel, vol. 62 (1960), pp. 1146—52.

50 ALEX MAZEL, Primary Examiner.

R. T. GALLAGHER, Assistant Examiner.

U.S. CL. X.R.

260—23.3